

# UNITED STATES PATENT OFFICE.

ROY LINDEN HILL, OF TAMAQUA, PENNSYLVANIA, ASSIGNOR TO ATLAS POWDER COMPANY, OF WILMINGTON, DELAWARE, A CORPORATION OF DELAWARE.

## EXPLOSIVE MIXTURE.

1,360,397.

Specification of Letters Patent. Patented Nov. 30, 1920.

No Drawing. Original application filed August 30, 1918, Serial No. 252,029. Divided and this application filed July 25, 1919, Serial No. 313,246. Renewed October 8, 1920. Serial No. 415,673.

To all whom it may concern:

Be it known that I, Roy L. Hill, a citizen of the United States of America, residing at Tamaqua, in the county of Schuylkill and State of Pennsylvania, have invented certain new and useful Improvements in Explosive Mixtures, of which the following is a specification.

This application is a division of my co-pending application Serial Number 252,029, filed Aug. 30, 1918 and is filed to claim specifically certain of the ingredients used in my new explosive mixture. As is clearly disclosed in my copending application aforesaid my composition as a whole consists principally of the following ingredients combined substantially in the following proportions:

|    |                                                                                                         |           |
|----|---------------------------------------------------------------------------------------------------------|-----------|
| 20 | Ammonium perchlorate (water proofed or otherwise)                                                       | 45 to 55% |
|    | Nitro-starch                                                                                            | 35 to 45% |
|    | Compounds or mixtures of compounds containing a metal or metals which will readily combine with chlorin | 0 to 10%  |
| 25 | An oil or other liquid to prevent dustiness                                                             | 0 to 5%   |

Ammonium perchlorate contains an excess of oxygen over that needed theoretically for its combustion of about twenty-seven per cent.; further, in nitro-starch there is not enough oxygen for complete combustion, the deficiency varying inversely with the extent to which the starch has been nitrated. The two substances, properly combined, will in themselves make a mixture of very high explosive force. However, such a mixture alone would develop, on detonation, chlorin and hydrochloric acid which would be objectionable except in very open work. I propose to remedy this condition by the well known method of adding a compound or mixture of compounds of a metal or metals which will readily combine with chlorin. For this I have used such substances as sodium nitrate and manganese dioxid, but I do not limit myself to these two compounds. Such substances have been used before with chlorin-containing explosive mixtures, but never, so far as I know, in combination with nitro-starch and ammonium perchlorate.

55 That my explosive may not be so dry and

dusty as to offer difficulties in mixing, packing, using and the like, I propose to mix with it some oil or other liquid. I have used for this purpose castor oil, coal tar distillates and liquid nitro-aromatic compounds, such as nitrated solvent naphtha, but I do not limit myself to these substances.

The ingredients of my explosive may be prepared and mixed in any of the well known ways, including their "water-proofing" with paraffin, petrolatum, waxes and the like; and my explosive may be packed in the usual types of high explosive cartridges or in any other suitable container.

Most non-freezing explosives which have been made or proposed have the objection of low "sensitiveness" with the tendency to become very "insensitive" in keeping or "aging." To eliminate this tendency several methods have been suggested by others, for instance, the use of metallic powders, especially aluminum and zinc dusts, but there is a question as to the safety of this.

My explosive offers the advantage of relatively high "sensitiveness," of very high explosive strength, of controllable density, and ease of mixing.

I put especial stress on the high explosive strength, of my non-freezing mixture, since I can obtain over 80% weight strength and over 70% bulk strength, compared with so-called straight nitro-glycerin explosives.

In order that anyone familiar with the manufacture of explosives may understand how my new explosive mixture may be made up, I will give the composition of a mixture which has given excellent results on tests.

|                                                         |     |
|---------------------------------------------------------|-----|
| Ammonium perchlorate                                    | 50% |
| Nitro-starch                                            | 40% |
| Sodium nitrate, coated with one per cent. of petrolatum | 8%  |
| Nitrated "solvent naphtha"                              | 2%  |
|                                                         | 100 |

It should be understood that this example is for illustrative purposes merely, and that my invention is not limited to this one exact mixture.

I have also found that other proportions of ammonium perchlorate and nitro-starch may be used, and that many other substances may be added, either to decrease the explosive strength of the mixture where a lower strength explosive is desired, to ob-

tain desired densities, or to obtain varied rates of detonation, or varied sensitiveness, or for other purposes. In such mixtures, in combination with the ammonium perchlorate and nitro-starch in varying proportions, I have used such substances as dinitrotoluene, trinitrotoluene, sulfur, wood meal, or other similar diluent substances, various liquid or solid nitro aromatic substances, other combustible and incombustible and water proofing or plasticizing substances such as waxes or paraffins, various oils and the like. To avoid or decrease the formation of objectionable fumes of chlorin or hydrochloric acid after explosion, I have used compounds or mixtures of compounds of a metal or metals which will readily combine with chlorin, which are not new with explosive mixtures containing chlorates or perchlorates, but which to my knowledge have never been used or described in combination with mixtures containing essentially ammonium perchlorate and nitro-starch.

Another mixture that I have found to give excellent results is as follows:

|                          |     |
|--------------------------|-----|
| Ammonium perchlorate     | 36% |
| Nitro-starch             | 32% |
| Manganese dioxid         | 6%  |
| Sodium nitrate           | 20% |
| 30 Sulfur                | 4%  |
| Nitrated solvent naphtha | 2%  |

Having thus clearly set forth the essential features of my invention, and shown by example how it may be applied, I do claim and desire to secure by Letters Patent based on 35 this particular divisional application—

1. An explosive mixture, consisting of ammonium perchlorate and nitro-starch; combined with an oil. 40
2. An explosive mixture, consisting of ammonium perchlorate, forty-five to fifty-five per cent. and nitro-starch, thirty-five to forty-five percent.; combined with an oil up to five per cent. 45
3. An explosive mixture consisting of ammonium perchlorate, nitro-starch and a liquid nitro-aromatic compound. 50
4. An explosive mixture consisting of ammonium perchlorate, forty-five to fifty-five per cent. nitro-starch, thirty-five to forty-five per cent. and a liquid nitro-aromatic compound up to five per cent. 55
5. An explosive mixture comprising ammonium perchlorate nitro-starch and a water proofing ingredient.

In testimony whereof I affix my signature in the presence of two witnesses.

ROY LINDEN HILL.

Witnesses:

R. M. COOK,  
C. D. PRATT.